

1

3,242,130

## PHOSPHORODITHIOIC ZINC SALT BASED CORROSION INHIBITING COMPOSITION COMPRISING AN EPOXY RESIN, ACYLATED POLYAMINE AND FILLER

Le Roy G. Jackopin, Painesville, Ohio, assignor to The Lubrizol Corporation, Wickliffe, Ohio, a corporation of Ohio

No Drawing. Filed Nov. 9, 1961, Ser. No. 151,195  
6 Claims. (Cl. 260—32.8)

The present invention relates to a fluid composition adapted to provide an electrically-conductive, protective coating for metals. In a more particular sense, it relates to a fluid composition adapted to provide a weldable protective coating for ferrous metals.

It is common practice in the automotive industry to coat various ferrous undercarriage parts of passenger cars and trucks such as brackets, box-channels, panels, and braces, with a suspension of zinc dust in an organic vehicle, generally an alkyd or synthetic resin. Some manufacturers depart from this practice by coating ferrous metal stock with the zinc-filled organic vehicle before it is formed into the various parts. In any event, they all seek to provide these ferrous parts with a coating which protects them from corrosion and which, at the same time, does not impair the weldability of the coated ferrous surface. In addition the coating must be sufficiently hard and adherent so that it will withstand forming operations without scoring or flaking.

The zinc-filled organic vehicles, i.e., "zinc-filled paints," presently available for this purpose have not been fully satisfactory. They have afforded only limited protection against corrosion although they have been satisfactory with respect to weldability. In an effort to improve corrosion resistance, some manufacturers have first treated the ferrous parts and/or ferrous stock from which the parts are made with an aqueous phosphating solution to form thereon an inorganic phosphate coating and thereafter applied a zinc-filled paint over the phosphate coating. Although a significant improvement in corrosion resistance is obtained by such a two-step procedure, the increased handling and processing costs have seriously limited its widespread application.

It is an object of the present invention to provide a fluid composition which forms a protective, adherent, easily weldable coating on metal surfaces.

Another object is to provide a composition particularly adapted to prevent the corrosion of ferrous metal surfaces.

Still another object is the provision of corrosion-resistant, weldable ferrous articles.

According to the present invention, these and other objects are achieved by means of a fluid composition adapted to form a protective coating on metals which contains as essential ingredients (A) finely-divided zinc, (B) an epoxy resin, (C) a polyvalent metal salt of the phosphorodithioic acid prepared by the reaction of a mixture of monohydric and polyhydric alcohols with a phosphorus sulfide, and (D) an oil-soluble acylated amine prepared by the reaction of a substituted succinic compound selected from the class consisting of substituted succinic acids having the structural formula



2

and substituted succinic anhydrides having the structural formula



in which structural formulas R is a large, substantially aliphatic hydrocarbon radical having at least about 50 carbon atoms, with more than an equivalent amount of an amine selected from the group consisting of alkylene amines and hydroxyalkyl substituted alkylene amines.

In general the fluid composition will also contain a viscosity-reducing amount of a volatile solvent and a pigment-suspending agent such as castor wax or a polyvalent metal stearate to prevent the settling and agglomeration of the zinc dust into a hard, difficultly-dispersible precipitate.

## INGREDIENT (A)

Ingredient (A), the finely divided zinc, is preferably commercial powdered zinc passing 325-mesh screen according to ASTM Test E 11-58 T. Powdered zinc of such fineness is more readily dispersed with the other ingredients of the composition than is a coarser grade and, furthermore, shows less tendency to precipitate upon storage.

## INGREDIENT (B)

Ingredient (B), the epoxy resin, is any one of a number of well-known organic resins which are characterized by the presence therein of an epoxide group, i.e.,



where x is zero or a small whole number. In the last decade, a wide variety of such resins have become available commercially.

Such resins have either a mixed aliphatic-aromatic or an exclusively non-benzenoid (i.e., aliphatic or cycloaliphatic) molecular structure.

The mixed aliphatic-aromatic epoxy resins which are preferred for the purpose of the present invention are generally prepared by the well-known reaction of a bis(hydroxyaromatic)alkane or a tetrakis(hydroxyaromatic)alkane with a halogen-substituted aliphatic epoxide in the presence of a base such as, e.g., sodium hydroxide or potassium hydroxide. Under these conditions, hydrogen halide is first eliminated and the aliphatic epoxide group is coupled to the aromatic nucleus via an ether linkage. Then the epoxide groups condense with the hydroxyl groups to form polymeric molecules which vary in size according to the relative proportions of reactants and the reaction time. The following equations, using for purposes of illustration, epichlorohydrin and 2,2-bis(p-hydroxyphenyl)propane as reactants, are believed to represent some of the principal reactions which occur. They do not necessarily represent all reactions, however, and it is preferred to define the epoxy resins in terms of their starting materials and average molecular weight.





(iv) III may likewise condense with additional epichlorohydrin and 2,2-bis-(p-hydroxyphenyl)propane to form higher polymers of the postulated general structure:



wherein  $z$  is an integer from 2 to, e.g., about 50.

In lieu of the epichlorohydrin, one can use halogen-substituted aliphatic epoxides containing 4 or more carbon atoms, generally 4 to 20 carbon atoms, such as, e.g., 4-chloro-1,2-epoxybutane, 5-bromo-1,2-epoxypentane, 6-chloro-1,3-epoxyhexane, 8-iodo-1,2-epoxyoctane, 7-chloro-2,3-epoxyoctane, 8-bromo-2,4-epoxynonane, 7,8-dichloro-1,2-epoxydecane, 16-bromo-1,2-epoxyhexadecane, 20-iodo-16-keto-1,2-epoxyeicosane, 14-chloro-1,2,5,6-diepoxytetradecane, and the like. In general it is preferred to use a chlorine substituted terminal alkylene oxide (terminal denoting that the epoxide group is on the end of the alkyl chain) and a particular preference is expressed for epichlorohydrin by reason of its cheapness, commercial availability, and excellence in forming epoxy resins useful for the purpose of this invention.

If desired, the halogen substituted aliphatic epoxide may also contain substituents such as, e.g., hydroxy keto, nitro, nitroso, ether, sulfide, carboalkoxy, etc.

Similarly, in lieu of the 2,2-bis-(p-hydroxyphenyl)propane, one can use bis-(hydroxyaromatic)alkanes containing 16 or more carbon atoms, generally 16 to 30 carbon atoms such as, e.g., 2,2-bis-(1-hydroxy-4-naphthyl)propane; 2,2-bis-(o-hydroxyphenyl)propane; 2,2-bis-(p-hydroxyphenyl)butane, 3,3-bis-(p-hydroxyphenyl)hexane; 2-(p-hydroxyphenyl)-4-(1-hydroxy-4-naphthyl)octane, 5,5-bis-(p-hydroxy-o-methylphenyl)decane, bis-(p-hydroxyphenyl)methane, 2,2-bis-(p-hydroxy-o-isopropylphenyl)propane, 2,2-bis-(o,p-dihydroxyphenyl)propane, 2-(p-hydroxyphenyl)-5-(o-hydroxyphenyl)hexadecane, and the like. If desired, the bis-(hydroxyaromatic)alkane may contain substituents such as, e.g., halogen, nitro, nitroso, ether, sulfide, carboalkoxy, etc. In general, it is preferred to use a bis-(p-hydroxyphenyl)alkane since compounds of this type are readily available from the well-known condensation of phenols with aliphatic ketones or aldehydes in the presence of a dehydrating agent such as sulfuric acid. A particular preference is expressed for 2,2-bis-(p-hydroxyphenyl)propane, commonly referred to in the trade as "Bisphenol A," by reason of its low cost and commercial availability.

Epoxy resins which are especially suited for the purpose of the present invention are prepared by the reaction of a bis-(hydroxyphenyl)alkane, preferably 2,2-bis-(p-hydroxyphenyl)propane with a chlorine substituted terminal alkylene oxide, preferably epichlorohydrin, to produce a product having an average molecular weight within the range of 300 to 500 and preferably 350 to 400. One of such preferred epoxy resins having an average molecular weight of about 380 and prepared from 2,2-bis-(p-hydroxyphenyl)propane and epichlorohydrin is known by the trade designation "Epon 820." A related type of epoxy resin having an average molecular weight of about 616 and prepared from epichlorohydrin and symmetrical tetrakis-(p-hydroxyphenyl)ethane is available under the trade designation "Epon 1031."

Another general class of epoxy resins which are useful for the purpose of the present invention are the aliphatic or cycloaliphatic epoxy resins. These resins, which are

10 devoid of benzenoid rings, are of relatively recent origin. They are made commercially by oxidizing (generally by means of peracetic acid) various monomeric or polymeric



cyclic or acyclic olefins such as, e.g., methylcyclohexene, vinylcyclohexene, alpha-methyl-vinylcyclohexene, polybutadiene, etc., which contain at least one carbon-to-carbon multiple bond. One of such non-benzenoid epoxy resins, known by the trade designation "Oxiron 2001," is made by oxidizing polybutadiene with peracetic acid. It is useful as the epoxy resin ingredient of a composition of the present invention. It is likewise useful when blended with a mixed aliphatic-aromatic epoxy resin of the type described earlier.

#### INGREDIENT (C)

Ingredient (C), the polyvalent metal salt of a phosphorodithioic acid prepared by the reaction of a mixture of monohydric and polyhydric alcohols with a phosphorus sulfide, is described in detail in U.S. Patent 2,861,907, owned by the assignee of the present application. In the interest of not unduly lengthening the present specification, it is intended that the entire disclosure of this patent be 20 incorporated herein by reference. In brief, the patent describes the reaction of a mixture of a monohydric alcohol and from 0.25 to 4.0 equivalents of a polyhydric alcohol with a phosphorus sulfide, preferably  $\text{P}_2\text{S}_5$ , to form a complex phosphorodithioic acid which is then converted to a polyvalent metal salt by conventional methods.

The monohydric alcohols contemplated as reactants in the preparation of Ingredient (C) of this invention include principally alkanols, although alcohols such as phenethyl and benzyl alcohols likewise may be used. For the most part, however, such alkanols as ethyl, butyl, hexyl, octyl, decyl, dodecyl, etc., alcohols are contemplated as the monohydric alcohol reactant. A particularly preferred subclass of monohydric alcohols are the octyl alcohols.

The polyhydric alcohol reactant may be selected from the various dihydric, trihydric, tetrahydric, and higher polyhydric alcohols. Illustrative examples of such polyhydric alcohols include ethylene glycol, propylene glycol, butylene glycol, glycerol, pentaerythritol, butenediol, butyediol, etc. It is contemplated likewise to employ polyhydric alcohols which contain aromatic substituents.

The proportions of monohydric and polyhydric alcohols which are to be used in the preparation of Ingredient (C) are governed by considerations of solubility and fluidity on the one hand, and of satisfactory film-forming properties on the other hand. It has been found that the use of a disproportionately large amount of polyhydric alcohol in the reaction mixture results in a product which is too insoluble and intractable to allow convenient application to a metal surface. If the proportion of polyhydric alcohol used in the reaction mixture is below a certain minimum quantity, then the resulting product, although sufficiently fluid and soluble in many solvents, is not a satisfactory film-forming material. In view of these observations, it has been determined that the amount of polyhydric alcohol which can be used satisfactorily in the preparation of Ingredient (C) is within the range of 0.25 to 4.0 equivalents per equivalent of monohydric alcohol present in the reaction mass. It is particularly preferred to employ approximately equivalent amounts of monohydric and polyhydric alcohol reactants. The term

"equivalent" as used above is based upon a consideration of the number of hydroxyl groups in the particular alcohol reactant. Thus the equivalent weight of ethylene glycol is 31, one-half of the molecular weight thereof. The equivalent weight of pentaerythritol is 34, one-fourth the molecular weight thereof.

The reaction by which phosphorodithioic acids are prepared is well-known. It involves the reaction of one mole of phosphorus pentasulfide with 4 equivalents of an alcohol or mixture of alcohols. Lesser or greater amounts of alcohol can be used, of course, but in such instances there is either incomplete reaction or an excess of the alcohol remains as a diluent in the final product.

The metal constituent of Ingredient (C) is a polyvalent metal such as, e.g., barium, calcium, strontium, magnesium, zinc, cadmium, iron, manganese, lead, tin, nickel, cobalt, chromium, beryllium, etc. The divalent metals are preferred, and of these zinc is particularly preferred. These metal salts are prepared from the phosphorodithioic acid, generally by neutralization thereof with the particular basic metal compound of the desired metal. Thus the preparation of a zinc phosphorodithioate may be effected by the neutralization of the phosphorodithioic acid with zinc oxide. Similarly a barium salt may be prepared by neutralization with barium hydroxide octahydrate. Other methods of formation of such polyvalent metal salts may be accomplished by reaction of the phosphorodithioic acid with the free metal, or by the metathesis of a monovalent metal phosphorodithioate such as a sodium or potassium phosphorodithioate with a soluble metal salt, e.g., a chloride or nitrate, of the polyvalent metal.

Polyvalent metal phosphorodithioates disclosed in the patent and useful for the purpose of the present invention are shown in Table 1:

TABLE 1

| Example No.<br>of U.S.<br>2,861,907 | Polyvalent metal phosphorodithioate |                                             |                  |                                        |
|-------------------------------------|-------------------------------------|---------------------------------------------|------------------|----------------------------------------|
|                                     | Metal                               | Phosphorodithioic acid preparation          |                  |                                        |
|                                     |                                     | Alcohol                                     | Equiva-<br>lents | Moles<br>P <sub>2</sub> S <sub>5</sub> |
| 1.                                  | Zn.                                 | n-Octyl alcohol                             | 8                |                                        |
| 2.                                  | Zn.                                 | 1,2-propylene glycol                        | 8                | 4                                      |
| 3.                                  | Zn.                                 | Isooctyl alcohol                            | 4                |                                        |
| 4.                                  | Zn.                                 | 2-butene-1,4-diol                           | 4                |                                        |
| 5.                                  | Zn.                                 | Isooctyl alcohol                            | 2.94             |                                        |
| 6.                                  | Zn.                                 | 2-butene-1,4-diol                           | 2.94             | 1.45                                   |
| 7.                                  | Zn.                                 | Isooctyl alcohol                            | 5.0              |                                        |
| 8.                                  | Zn.                                 | Dipropylene glycol                          | 15.0             |                                        |
| 9.                                  | Zn.                                 | Isooctyl alcohol                            | 12               |                                        |
| 10.                                 | Zn.                                 | Dipropylene glycol                          | 12               | 6                                      |
| 11.                                 | Zn.                                 | n-Butyl alcohol                             | 10               |                                        |
| 12.                                 | Zn.                                 | Diethylene glycol                           | 10               |                                        |
| 13.                                 | Zn.                                 | C <sub>12</sub> alcohols                    | 6                |                                        |
| 14.                                 | Zn.                                 | Diethylene glycol                           | 6                | 3                                      |
| 15.                                 | Fe.                                 | Isooctyl alcohol                            | 12               |                                        |
| 16.                                 | Zn.                                 | Dipropylene glycol                          | 12               |                                        |
| 17.                                 | Zn.                                 | n-Octyl alcohol                             | 7.5              |                                        |
| 18.                                 | Zn.                                 | Diethylene glycol                           | 6                |                                        |
| 19.                                 | Zn.                                 | Glycerol                                    | 1.5              | 3.75                                   |
| 20.                                 | Zn.                                 | n-Octyl alcohol                             | 8                |                                        |
| 21.                                 | Zn.                                 | Glycerol                                    | 8                | 4                                      |
| 22.                                 | Zn.                                 | Isooctyl alcohol                            | 8                | 2.5                                    |
| 23.                                 | Zn.                                 | Pentaerythritol                             | 2                |                                        |
| 24.                                 | Zn.                                 | Isooctyl alcohol                            | 12               |                                        |
| 25.                                 | Zn.                                 | Diethylene glycol                           | 12               | 6                                      |
| 26.                                 | Zn.                                 | Isooctyl alcohol                            | 10               |                                        |
| 27.                                 | Zn.                                 | Neopentyl glycol                            | 10               |                                        |
| 28.                                 | Zn.                                 | Isooctyl alcohol                            | 4                |                                        |
| 29.                                 | Zn.                                 | 2,2-bis(4-beta-hydroxyethoxyphenyl) propane | 4                | 2                                      |
| 30.                                 | Ba.                                 | Isooctyl alcohol                            | 12               |                                        |
| 31.                                 | Ba.                                 | Diethylene glycol                           | 12               | 6                                      |
| 32.                                 | Ca.                                 | Isooctyl alcohol                            | 12               |                                        |
| 33.                                 | Ca.                                 | Dipropylene glycol                          | 12               |                                        |
| 34.                                 | Cd.                                 | Isooctyl alcohol                            | 8                |                                        |
| 35.                                 | Cd.                                 | Propylene glycol                            | 8                | 4                                      |
| 36.                                 | Pb.                                 | Isooctyl alcohol                            | 8                |                                        |
| 37.                                 | Pb.                                 | Propylene glycol                            | 8                | 4                                      |

For the purpose of the present invention the zinc phosphorodithioates are preferred and a particular preference is expressed for the low-cost zinc salt of the phosphorodithioic acid prepared by the reaction of equivalent amounts of isoctyl alcohol and dipropylene glycol with

phosphorus pentasulfide as specifically described in Example 5 of U.S. Patent 2,861,907.

In some instances, zinc phosphorodithioates prepared from mixtures of monohydric and polyhydric aromatic alcohols (i.e., phenols) are also useful as Ingredient (C) of this invention. Specifically illustrative of the preparation of this type of zinc phosphorodithioate is the following:

*Example C-1*

In a flask equipped with a stirrer, 576 grams (3 moles) of heptylphenol and 114 grams (0.5 mole) of 2,2-bis(p-hydroxyphenyl)propane are introduced and heated to 120° C. While the whole is stirred vigorously, 222 grams (1 mole) of P<sub>2</sub>S<sub>5</sub> is added gradually over a period of 3 hours and heating is continued for an additional 3 hours. Filtration of the mass yields the desired complex phosphorodithioic acid, which is diluted with an equal weight of toluene to facilitate handling.

1376 grams of the toluene solution of the acid is mixed with 75 grams of zinc oxide and 5 grams of water. The whole is heated for 5 hours at 60-65° C. and then filtered to yield a filtrate which is a 51.2% solution of the desired zinc phosphorodithioate in toluene. It contains 2.99% of phosphorus, 6.31% of sulfur, and 3.34% of zinc.

INGREDIENT (D)

Ingredient (D), the oil-soluble acylated amine, is described in detail in the copending application of W. M. Le Suer et al., Serial No. 802,667, filed March 30, 1959, now U.S. Patent 3,172,892, and owned by the assignee of the present application. In the interest of not unduly lengthening the present specification it is intended that the disclosure of the said Le Suer et al. application, particularly the portion thereof which deals with species of acylated amines derived from the reaction of a substituted succinic compound with more than an equivalent amount of an ethylene amine, be considered as forming a part of the present specification.

In summary, Serial No. 802,667 deals with mixing a substituted succinic compound selected from the class consisting of substituted succinic acids having the structural formula



45 and substituted succinic anhydrides having the structural formula



50 in which structural formulas R is a large, substantially aliphatic hydrocarbon radical having at least about 50 carbon atoms, with at least about one-half an equivalent amount of an ethylene amine, and heating the resulting mixture to effect acylation and remove the water formed thereby.

The size of the substituent on the succinic acid or anhydride is of importance in the preparation of Ingredient (D) because it allows the preparation of a product which 60 satisfies the objects of this invention. It is important that this substituent be large, that it have at least about 50 carbon atoms in its structure. These substituent groups are substantially aliphatic hydrocarbon radicals including both alkyl and alkenyl radicals. They are commonly derived from polyolefins such as polyethylene, polypropylene, polybutene, polyamylene, etc., although they may be derived from any substantially aliphatic hydrocarbon.

The substituted succinic acids and anhydrides which 70 are contemplated as a reactant in the process for the preparation of Ingredient (D) are readily available from the reaction of maleic anhydride with a high molecular weight olefin or a chlorinated high molecular weight olefin. The product from such a reaction is the corresponding alkenyl succinic anhydride. The reaction involves merely heating these two reactants at a tempera-

ture of about 150 to 200° C. The reactants in each case are illustrated by the following equations:



It will be appreciated that the reactions may not go precisely as indicated above, especially with respect to the particular carbon atom of the olefin or chloride reactant which ultimately becomes attached to the maleic acid or anhydride reactant, but other than this the equations are believed to be illustrative. Furthermore, although the product of this reaction has been indicated as being an alkenyl succinic anhydride; it is apparent that similar products can be prepared by this process in which the substituent is something other than an alkenyl group. For the purpose of the present invention this substituent should, however, be substantially aliphatic group and in most cases, of course, it will be an alkyl or alkenyl group. In some cases, however, it may well be desirable to employ a substituted succinic anhydride in which the substituent is derived from a copolymer of styrene and isobutylene, or of a substituted styrene and some other aliphatic olefin. In these cases copolymer will be substantially aliphatic, that is, the composition of the copolymer will be predominantly aliphatic.

The most commonly used sources of the substantially aliphatic hydrocarbon substituents are the polyolefins. These are illustrated by polyethylene, polypropylene, polyisobutene, etc. A particularly preferred polyolefin for this use is polyisobutene. Thus the condensation of a polyisobutene having a molecular weight of about 750 with maleic anhydride yields an alkenyl succinic anhydride which upon further reaction with an ethylene amine produces a material which is particularly effective as Ingredient (D) of the present invention.

The substituted succinic anhydride ordinarily is reacted directly with the ethylene amine, although in some instances it may be desirable first to convert the anhydride to the acid before reaction with the ethylene amine. In other circumstances it may be desirable to prepare the substituted succinic acid by some other means and to use an acid prepared by such other means in the process. In any event, either the acid or the anhydride may be used in the preparation of Ingredient (D).

The term "ethylene amine" is used in a generic sense to denote a class of polyamines conforming for the most part to the structure:



in which  $x$  is an integer and R is a low molecular weight alkyl radical or hydrogen. Thus it includes, for example, ethylene diamine, diethylene triamine, triethylene tetramine, tetraethylene pentamine, pentaethylene hexamine, etc. These compounds are discussed in some detail under the heading "ethylene amines" in "Encyclopedia of Chemical Technology," Kirk and Othmer, volume 5, pages 898-905, Interscience Publishers, New York (1950). Such compounds are prepared most conveniently by the reaction of ethylene dichloride with ammonia. This process results in the production of somewhat complex mixtures of ethylene amines, including cyclic condensation products such as piperazines, and these mixtures find use in the preparation of Ingredient (D). On the other hand, quite satisfactory products may be obtained also by use of pure ethylene amines. An especially useful ethylene amine for reasons of economy as well as effectiveness is a mixture of ethylene amines prepared by the reaction of ethylene chloride and ammonia, having a composition which corresponds to that of tetraethylene pent-

amine. This is available in the trade under the trade name "Polyamine H."

It has been noted that more than a chemically equivalent amount of the ethylene amine per equivalent of substituted succinic compound should be used to produce a product which is satisfactory as Ingredient (D). Amounts of the ethylene amine ranging from about 1.1 to about 8 equivalents, preferably from about 1.5 to about 4 equivalents, per equivalent of substituted succinic compound are generally used. Amounts greater than 8 equivalents of ethylene amine per equivalent of substituted succinic compound may also be used if desired, but there appears to be no advantage in the use of such large amounts of the ethylene amine reactant. The chemical equivalency of the ethylene amine reactant is based upon the nitrogen content, i.e., one having 4 nitrogens per molecule has 4 equivalents per mole.

In the preparation of Ingredient (D), the ethylene amine and the substituted succinic compound are mixed and heated at a temperature within the range of about 80° C. to about 200° C., preferably 100° C. to 160° C., until most or all of the water of reaction has been removed. Thus a useful method of carrying out this step is to add some toluene to the reaction mixture and remove the water of reaction by azeotropic distillation.

It has been found that in lieu of the ethylene amine reactant, one can use for the purpose of the present invention any alkylene amine or hydroxyalkyl substituted alkylene amine reactant conforming for the most part to the structure



in which  $n$  is an integer, A is hydrogen, a hydrocarbon radical, or a hydroxyalkyl radical, and Q is a divalent aliphatic radical containing at least 2 carbon atoms. The A substituents in the above formula can also be considered as forming a divalent alkylene radical, in which instance a cyclic structure results. Q is generally an alkylene radical such as ethylene, trimethylene, tetramethylene, etc., although in certain instances it may be an aliphatic radical which contains ether or sulfide substituents such as, e.g., an -alkylene-O-alkylene- or -alkylene-S-alkylene-radical.

Specific examples of such amine reactants are trimethylene diamine, di-(trimethylene)triamine, tris-(trimethylene)tetramine, tri-(hexamethylene)tetramine, decamethylene diamine, N-octyl trimethylene diamine, N,N'-diocetyl trimethylene diamine, N-(2-hydroxyethyl)ethylene diamine, piperazine, 1-(2-aminopropyl)piperazine, 1,4-bis-(2-aminoethyl)piperazine, 1-(2-hydroxyethyl)piperazine, di-(hydroxypropyl-substituted)tetraethylene pentamine, N-(3-hydroxypropyl)tetramethylene diamine, pyrimidine, 2-methyl-imidazoline, and 1,3-bis-(2-aminoethyl)imidazoline.

Specific examples of acylated amines which are disclosed in detail in Serial No. 802,667 and which are useful as Ingredient (D) are shown in Table 2:

TABLE 2

| Example No.<br>of Serial No.<br>802,667 | Acylated amine prepared from—                                            |                  |                                                                                      |                  |
|-----------------------------------------|--------------------------------------------------------------------------|------------------|--------------------------------------------------------------------------------------|------------------|
|                                         | Succinic com-<br>pound                                                   | Equiv-<br>alents | Amine                                                                                | Equiv-<br>alents |
| 3-----                                  | Polyisobutene<br>(mol. wt. 850)<br>substituted<br>succinic<br>anhydride. | 1.0              | An ethylene<br>amine mix-<br>ture cor-<br>responding to<br>triethylene<br>tetramine. | 1.5              |
| 4-----                                  | do-----                                                                  | 1.0              | Triethylene<br>tetramine.                                                            | 1.5              |
| 5-----                                  | do-----                                                                  | 0.78             | "Polyamine<br>H,"                                                                    | 1.55             |
| 6-----                                  | do-----                                                                  | 1.0              | Ethylen-<br>e diamine.                                                               | 1.5              |

Additional examples of acylated amines useful as ingredient (D) are as follows:

*Example D-1*

A polyisobutene-substituted succinic anhydride is prepared by the reaction of a chlorinated polyisobutene (ca. 4% chlorine content) with maleic anhydride at 200° C. The polyisobutene has an average molecular weight of 850 and the resulting alkenyl succinic anhydride is found to have an equivalent weight of about 515. A mixture of 3 parts of triethylene tetramine and 1 part of diethylene triamine, by weight, in the amount of 279 grams (7.76 equivalents based on nitrogen) is added to a solution of 1000 grams (1.94 equivalents) of the alkenyl succinic anhydride in 200 grams of toluene over a period of 4 minutes at 57-88° C. After the initial exothermic reaction subsides, the whole is heated for 5 hours at 155° C. The water of reaction is collected in a side arm water trap and amounts to about 26 grams. The reaction mass is then stripped of solvent by heating at 160° C./5 mm. Hg until distillation ceases. The residue is an acylated amine having a nitrogen content of 7.54%.

*Example D-2*

In a manner like that described in Example D-1, 249 grams (4 equivalents based on nitrogen) of bis-(3-aminopropyl)amine is mixed with a solution in 266 grams of toluene of 920 grams (1.33 equivalents) of a polyisobutene-substituted anhydride having an equivalent weight of about 690. The whole is heated for 6 hours under reflux and then heated to 220° C./3 mm. Hg to remove the solvent. The residue is an acylated amine having a nitrogen content of 4.0%.

*Example D-3*

In a manner like that described in Example D-1, 333 grams (3.78 equivalents based on nitrogen) of bis-(3-aminopropyl)ether of ethylene glycol is reacted with 1000 grams (1.89 equivalents) of a polyisobutene substituted succinic anhydride having an equivalent weight of about 530, using 300 grams of xylene as a reaction solvent. Upon removal of the xylene solvent the acylated amine remains as the residue. It contains 4% of nitrogen.

*Example D-4*

In a manner like that described in Example D-1, 418 grams (3.78 equivalents based on nitrogen) of bis-(3-aminopropyl)ether of diethylene glycol is reacted with 1000 grams (1.89 equivalents) of a polyisobutene substituted succinic anhydride having an equivalent weight of about 530, using 300 grams of toluene as a reaction solvent. Upon removal of the toluene solvent, the acylated amine remains as the residue. It contains 3.8% nitrogen.

*Example D-5*

In a manner like that described in Example D-1, 194 grams (3.74 equivalents based on nitrogen) of N-(2-aminoethyl)ethanolamine is reacted with 1000 grams (1.87 equivalents) of a polyisobutene substituted succinic anhydride having an equivalent weight of about 535, using 786 grams of toluene as a reaction solvent. Upon removal of the toluene solvent, the acylated amine remains as the residue. It contains 4.3% nitrogen.

Each of the Ingredients (A), (B), (C), and (D) are essential in preparing the fluid compositions of the present invention. In addition to these characterizing ingredients it is generally desirable to have present a small proportion of a pigment-suspending agent such as castor wax or a polyvalent metal stearate such as, e.g., zinc stearate, cadmium stearate, or aluminum stearate, to prevent the settling of Ingredient (A), the zinc dust, from the other ingredients of the coating composition. In most instances it is also desirable to dilute one or more of the characterizing ingredients or mixtures of two or more of such ingredients with a viscosity-reducing amount of a volatile solvent so as to facilitate the application of the coating composition to metal surfaces. Solvents useful for this purpose include those which are commonly

employed in the paint and lacquer industry such as, e.g., petroleum hydrocarbon solvents; alcohols such as, e.g., methyl, ethyl, propyl, butyl, and amyl alcohols; ketones such as, e.g., acetone, diethyl ketone, methyl isobutyl ketone, methyl ethyl ketone, etc.; the lower chlorinated alkanes such as, e.g., ethylene dichloride, 1,2-dichloropropane, butyl chloride, etc.; aromatic hydrocarbons such as, e.g., benzene, toluene, xylene, mesitylene, etc.; and aliphatic ether such as, e.g., diisopropyl ether, diisobutyl ether, and the like. In certain instances it is desirable to use mixtures of two or more solvents.

Although the proportions of the several ingredients are not particularly critical, best results from the standpoint of economy, ease of application, and weldability of the coated metal surface are obtained when one uses a composition prepared from a mixture of from about 125 to about 200 parts preferably from about 150 to about 175 parts, of Ingredient (A), the zinc dust; from about 10 to about 30 parts, preferably from about 14 to about 25 parts, of Ingredient (B), the epoxy resin; from about 4 to about 16 parts, preferably from about 6 to about 10 parts, of Ingredient (C), the complex polyvalent metal phosphorodithioate; and from about 5 to about 15 parts, preferably from about 8 to about 12 parts, of Ingredient (D), the oil-soluble acylated amine; all parts being by weight. To this mixture there may be added, optionally, a small amount, generally from about 1 to about 3 or 4 parts, of a pigment-suspending agent and at least about 25 parts, preferably from about 30 to about 70 parts, of a viscosity-reducing solvent. The use of a pigment-suspending agent, although not absolutely essential, is required if settling of the zinc dust is to be avoided. In the absence of this agent, the composition must be stirred at frequent intervals after preparation and during use. Thus, for obvious practical reasons, it is highly desirable to include a pigment-suspending agent in the compositions of this invention.

The order of mixing the ingredients of the composition is not critical when the composition is prepared for immediate use. It is generally most convenient, however, to mill the pigment-suspending agent, if one is to be used, in the solvent-diluted epoxy resin Ingredient (B) by means of a ball mill or other conventional paint-dispersing equipment. This mixture is then removed to another vessel equipped with means for stirring and Ingredients (C) and (D) are added and stirred well. A small proportion of solvent, either added directly to the vessel contents or present in Ingredients (C) and/or (D), serves to facilitate the mixing operation. After the mixture has been stirred for a sufficient time to become homogeneous, the zinc dust is added slowly while the whole is stirred vigorously. The consistency of the mass is then adjusted by the addition, if required, of a further amount of solvent so as to yield a composition which has a viscosity well-suited for the particular method by which it is to be applied to a metal surface. The application to a metal surface may be made by any one of the methods commonly used in the paint industry such as, e.g., dipping, brushing, roller-coating, or spraying.

If the composition is not to be used until quite some time after preparation, for example, if it is to be stored for a period longer than about one month before use, then Ingredients (C) and (D) should be stored apart from the other ingredients of the composition. Tests have shown that a complete composition has a tendency to set to an irreversible gel after having been stored for about one month in a sealed can. This gelation can be avoided, as indicated, by storing Ingredients (C) and (D) separately or admixed with each other and then adding them to the remaining ingredients shortly before the complete composition is to be used. Of course, in instances where the composition is to be used within, say, 3 weeks, no such storage precautions are necessary.

Although any of the various Ingredients (A) through (D) described earlier may be used in compounding the

composition of the present invention, certain ingredients and combinations thereof are preferred for reasons of their commercial availability and economy. Thus, for example, a very useful and economical group of compositions of this invention contain as essential ingredients (A) from about 125 to about 200 parts of powdered zinc, (B) from about 10 to about 30 parts of an epoxy resin of 300-500 average molecular weight prepared by the reaction of a bis-(p-hydroxyphenyl)alkane with a chlorine-substituted terminal alkylene oxide, (C) from about 4 to about 16 parts of a zinc salt of the phosphorodithioic acid prepared by the reaction of a mixture of a monohydric alcohol and from 0.25 to 4.0 equivalents of a polyhydric alcohol with phosphorus pentasulfide, (D) from about 5 to 15 parts of an oil-soluble acylated amine prepared by the reaction of a polyisobutene-substituted succinic anhydride with from about 1.5 to about 4 equivalents of an ethylene amine, and (E) at least about 25 parts of a volatile solvent.

A preferred sub-class of compositions in the above group include those compositions which contain as essential ingredients (A) from about 150 to about 175 parts of powdered zinc passing 325-mesh screen, (B) from about 14 to about 25 parts of an epoxy resin of 350-400 average molecular weight prepared by the reaction of 2,2-bis-(p-hydroxyphenyl)propane with epichlorohydrin, (C) from about 6 to about 10 parts of a zinc salt of a phosphorodithioic acid prepared by the reaction of a mixture of about equivalent amounts of isoctyl alcohol and dipropylene glycol with phosphorus pentasulfide, (D) from about 8 to about 12 parts of an oil-soluble acylated amine prepared by the reaction of a polyisobutene-substituted succinic anhydride where in the polyisobutene has an average molecular weight of about 750 with about 4 equivalents of a mixture of diethylene triamine and triethylene tetramine, and (E) from about 30 and about 70 parts of a volatile solvent consisting of a mixture of aromatic petroleum spirits and methyl isobutyl ketone.

The aromatic petroleum spirits useful in preparing the compositions of the present invention are available from various petroleum refiners. They generally boil in the range from about 300° to about 400° F. and have a Kauri-butanol value of from about 50 to about 125. An economical, commercially available mixture of aromatic petroleum spirits boils in the range 316-349° F. and has a Kauri-butanol value of about 91.

Specific illustrations of the preparation of compositions of this invention are as follows:

#### Example I

1.63 grams of a commercial grade of castor wax known as "Thixcin R" is dispersed in 19.34 grams of an epoxy resin prepared from 2,2-bis-(p-hydroxyphenyl)propane

TABLE 3

| Ex. No. | Zn dust,<br>gms. | Pigment suspending<br>agent |            | Epoxy resin              |          | PMP <sup>1</sup> |    | Acylated amine               |      | Solvent                                     |      |
|---------|------------------|-----------------------------|------------|--------------------------|----------|------------------|----|------------------------------|------|---------------------------------------------|------|
|         |                  | Identity                    | Gms.       | Identity                 | Gms.     | A                | B  | Identity                     | Gms. | Identity                                    | Gms. |
| IV      | 125              | Al stearate                 | 3          | Epon 1031                | 25       | 1                | 5  | Ex. D-2                      | 11   | Methyl ethyl ketone                         | 35   |
| V       | 190              | Zn stearate                 | 4          | Epon 820                 | 15       | 7                | 10 | Ex. D-1                      | 6    | Diisopropyl ether                           | 30   |
| VI      | 150              | Castor wax                  | 1.5        | Oxiron 2001              | 30       | 12               | 15 | Ex. D-3                      | 14   | Aromatic petroleum<br>spirits. <sup>2</sup> | 30   |
| VII     | 170              | Castor wax<br>Cd stearate   | 1.5<br>1.5 | Epon 820<br>Epon 1031    | 8<br>6   | 17               | 12 | Ex. D-5                      | 8    | Diethyl ketone                              | 20   |
| VIII    | 200              | Castor wax                  | 3          | Oxiron 2001<br>Epon 820  | 15       | 15               | 16 | Ex. D-4                      | 10   | Xylene                                      | 15   |
| IX      | 140              | Castor wax<br>Zn stearate   | 2<br>2     | Oxiron 2001<br>Epon 1031 | 20<br>10 | 18               | 8  | Ex. 5 of Ser.<br>No. 802,667 | 7    | Methyl isobutyl<br>ketone                   | 40   |
| X       | 165              | Castor wax                  | 2.5        | Epon 820<br>Epon 1031    | 20<br>5  | 9                | 10 | Ex. 3 of Ser.<br>No. 802,667 | 12   | Mesitylene                                  | 20   |
|         |                  |                             |            |                          |          |                  |    |                              |      | Ethylene dichloride                         | 10   |
|         |                  |                             |            |                          |          |                  |    |                              |      | Methyl isobutyl<br>ketone                   | 60   |

<sup>1</sup> PMP=Polyvalent metal phosphorodithioate. Col. A=Ex. No. in U.S. Patent 2,861,907. Col. B=grams employed.

<sup>2</sup> Boiling range, 316-349° F. and Kauri-butanol value of 91.

and epichlorohydrin and having an average molecular weight of about 380 (available commercially under the trade designation "Epon 820") and 19.34 grams of a solvent ("solvent X") consisting of a mixture of 2 parts of methyl isobutyl ketone and 1 part of commercial aromatic petroleum spirits boiling in the range of 316-349° F. and having a Kauri-butanol value of 91. After the castor wax has been thoroughly dispersed in the epoxy resin solvent solution (15 minutes is normally required when a conventional paint-shaking machine is used), the whole is transferred to a vessel equipped with a propeller-type stirring device. 10 grams of an 80% solution in solvent X of a complex zinc phosphorodithioate according to Example 5 of U.S. Patent 2,861,907 and 19.32 grams of a 50% solution in solvent X of the acylated amine of Example D-1 are added to the vessel and the whole is stirred vigorously until the ingredients form a homogeneous mass. Then, while stirring is continued, 163 grams of powdered zinc passing 325-mesh screen is added gradually to the vessel over a period of about 10 minutes. When the zinc powder is thoroughly dispersed in the liquid ingredients, the composition is ready for packaging or use.

#### Example II

In a manner like that described in Example I the following ingredients are blended to form a composition of the invention:

30 1.63 grams of Thixcin R  
30 14 grams of Epon 820  
30 14 grams of solvent X  
30 20 grams of an 80% solution in solvent X of the complex zinc phosphorodithioate of Example 5 of U.S. 2,861,907  
35 14 grams of a 50% solution in solvent X of the acylated amine of Example D-1  
163 grams of powdered zinc passing 325-mesh screen

#### Example III

In a manner like that described in Example I the following ingredients are blended to form a composition of the invention:

40 0.75 grams of Thixcin R dissolved in 87.75 grams of solvent X  
45 115.5 grams of Epon 820 dissolved in 115.5 grams of solvent X  
45 15.62 grams of the zinc phosphorodithioate-toluene product of Example C-1  
50 115.5 grams of a 50% solution in solvent X of the acylated amine of Example D-1  
978 grams of powdered zinc passing 325-mesh screen

Additional examples of compositions of the invention are shown in Table 3:

The compositions of this invention are generally applied to the metal surface to be protected in an amount sufficient to yield a dried film thickness of from about 0.5 to about 10 mils and preferably from about 1 to about 3 mils. After application to the metal surface, the composition may be dried by any one of the various methods commonly employed in the paint and lacquer field such as, e.g., air-drying at ambient temperature, drying in a current of hot air, baking in an oven, or baking under a bank of infrared lamps. Best results from the standpoint of good adherence, film hardness, and corrosion protection are obtained with the compositions of this invention when a film thereof is dried by a baking procedure. Oven-baking procedures call for exposure of the coated metal surface to temperature in the range of 250-450° F. for a period ranging from about 1 minute to about 1 hour. The lower baking temperatures generally require longer periods of time than the higher baking temperatures; for example, typical procedures call for baking at 400° F. for 2 minutes, or 15 minutes at 360° F. or 45 minutes at 250° F.

In most instances the compositions of this invention will be applied directly to the bare metal surface to be protected. In certain applications however, where superior corrosion resistance is sought, the metal may be pretreated with a metal passivating solution such as, e.g., a dilute chromic acid solution, or an aqueous phosphating solution such as, e.g., aqueous acidic zinc dihydrogen phosphate, aqueous acidic manganese dihydrogen phosphate, and the like. Such metal passivating or phosphating techniques are well-known and are described for example, in U.S. Patents 1,206,075, 1,247,668, 1,305,331, 1,485,025, 1,610,362, 1,980,518, 2,001,754, 2,901,385, 2,846,342, 2,868,682, 2,901,437, and 2,876,150. A very useful and effective class of aqueous phosphating solutions containing as essential ingredients zinc ion, phosphate ion, nitrate ion, and calcium ion are described in U.S. application Serial No. 373,449, filed August 5, 1953, now U.S. Patent 3,090,709, by John A. Henricks, and owned by the assignee of the present application.

In addition to pretreatment of the metal surface, it may also be desirable in certain instances, particularly where decorative effects are sought, to "top-coat" the dried film of a composition of this invention with a paint, paint primer, lacquer, or enamel. The compositions of this invention serve as an excellent base for such top-coats in that they inhibit the deterioration of the underlying base metal and thereby remove the principal cause of blistering, flaking, and other forms of loss of coating adhesion. The above discussion regarding pretreatment of the metal surface and top-coating of the dried film of the compositions of this invention is not to be construed as indicating that such pretreatments or post-treatments are at all re-

A number of tests were carried out to determine the efficacy of the present compositions, including tests to measure film hardness, adhesion, and corrosion prevention.

5 In all of the tests, 4-inch x 8-inch panels of clean, solvent-degreased, 20-gauge SAE 1020 cold-rolled steel prepared according to ASTM procedure D 609-52 were used to receive films of the coating compositions of this invention. The compositions were brushed on the steel panel and dried in the indicated manner to provide a film having a thickness of  $1.5 \pm 0.2$  mils. The prepared panels were then subjected to the tests described below, the results of which are given in Table IV.

15 *Sward film hardness.*—This test is carried out using a Model C Sward Rocker Hardness apparatus manufactured by Gardner Laboratory, Inc. In this test a dual metal wheel, weighted unequally and having a bladed periphery, is placed in contact with the surface to be tested at 60° F. The wheel is set in motion and the number of 20 swings (i.e., one-half the number of oscillations) of predetermined magnitude are counted. The harder the surface, the greater the number of swings. Conversely, the softer or the tackier the surface, the fewer the number of swings. Thus, the rating expressed in swings is a measure 25 of the relative hardness of the surface under test.

20 *Conical mandrel adhesion.*—The apparatus employed in this test is described in ASTM procedure D 522-41. In this test a 4-inch x 8-inch coated panel is placed in contact with a steel cone of fixed size and shape and then 25 bent 180° along its 4-inch dimension. The panel is removed from the bending apparatus and adhesive cellophane tape is applied to the coating on the bent portion of the panel. The tape is then rapidly removed and the percent of coating still adhering to the panel is estimated and 30 reported as "percent adhesion."

35 *Salt fog corrosion.*—The apparatus used for this test is described in ASTM procedure D 117-57T. It consists of a chamber in which a mist or fog of 5 percent aqueous sodium chloride is maintained in contact with 40 test panels for a predetermined time at  $95^\circ \pm 2$ ° F.

In the 120-hours test, the coating on the panel is pierced with a pointed instrument to yield a vertical scribe beginning one inch from the top of the panel and ending one 45 inch from the bottom thereof. The panel is then placed in a chamber for 120 hours and removed for inspection. The "creep rating" is the average loss of coating from each side of the scribe expressed as an integer which represents the number of thirty-seconds of an inch. The panel is also visually inspected for rust and the amount thereof 50 is reported as "percent of area rusted."

In the 250-hour test, an unscribed, coated panel is placed in the chamber for 250 hours then removed for inspection. The amount of rust is reported as "percent of area rusted."

TABLE 4

| Composition of Ex. No. | Sward film hardness            |        |                | Conical mandrel adhesion       |                  |                                   | Salt fog corrosion <sup>1</sup> |             |              |                                     | Remarks    |
|------------------------|--------------------------------|--------|----------------|--------------------------------|------------------|-----------------------------------|---------------------------------|-------------|--------------|-------------------------------------|------------|
|                        | Panel preparation <sup>1</sup> | Rating | Remarks        | Panel preparation <sup>1</sup> | Percent adhesion | Remarks                           | Panel preparation <sup>1</sup>  | Test, hours | Creep rating | Percent of area rusted <sup>2</sup> |            |
| I.....                 | A.....                         | 7      | Very good.     | A.....                         | 100              | Excellent.....                    | (B.....                         | 120         | 0            | { 1                                 | Very good. |
| II.....                | A.....                         | 7      | do             | A.....                         | 100              | { Very good; few hairline cracks. | (B.....                         | 250         | { 0          | { 0                                 | Excellent. |
| III.....               | { A.....<br>B.....<br>C.....   | 6      | Good.....      | A.....                         | 100              | Excellent.....                    | (B.....                         | 120         | 3            | { 5                                 | Good.      |
|                        |                                | 8      | Excellent..... |                                |                  |                                   | (B.....                         | 250         | 1            | { 5                                 | Do.        |
|                        |                                | 6      | Good.....      |                                |                  |                                   | (B.....                         | 120         | 0            | { 0                                 | Very good. |
|                        |                                |        |                |                                |                  |                                   | (B.....                         | 250         | 1            | { 0                                 | Excellent. |

<sup>1</sup> A = Film baked in an oven 2 minutes at 400° F.

B = Film baked in an oven 2 minutes at 400° F. and then 15 minutes at 360° F.

C = Film air-dried for 15 hours at room temperature.

<sup>2</sup> Inspection for rust does not include the so-called "white corrosion" which results from the conversion of the zinc powder to zinc salts and which is expected in zinc-filled paints that protect ferrous surfaces by the sacrificial consumption of zinc metal.

quired for adequate protection of metal surfaces. It has been offered merely to point out the versatility of the present compositions in adhering well to modified metal surfaces and in providing an excellent paint base in applications where a top-coat must be applied.

What is claimed is:

1. A fluid composition adapted to form a protective coating on metals which contains as essential ingredients (A) finely divided zinc, (B) an epoxy resin selected from the group consisting of aliphatic-aromatic, aliphatic, and

cycloaliphatic epoxy resins, (C) a polyvalent metal salt of the phosphorodithioic acid prepared by the reaction of a mixture of monohydric and polyhydric alcohols with a phosphorus sulfide, said polyvalent metal being selected from the group consisting of barium, calcium, strontium, magnesium, zinc, cadmium, iron, manganese, lead, tin, nickel, cobalt, chromium, and beryllium, and (D) an oil-soluble acylated amine prepared by mixing and heating at a temperature of from about 80° C. to about 200° C., a substituted succinic compound selected from the class consisting of substituted succinic acids having the structural formula



and substituted succinic anhydrides having the structural formula



in which structural formulas R is a large, substantially aliphatic hydrocarbon radical having at least about 50 carbon atoms, with more than an equivalent amount of amine of the structure



in which  $n$  is an integer, A is selected from the group consisting of hydrogen, a hydrocarbon radical, and a hydroxyalkyl radical, and Q is a divalent aliphatic radical containing at least 2 carbon atoms.

2. A composition in accordance with claim 1 further characterized in that the epoxy resin of (B) is prepared by the reaction of a bis(hydroxyaromatic) alkane with a halogen-substituted aliphatic epoxide.

3. A composition in accordance with claim 1 further characterized in that the polyvalent metal salt of (C) is a zinc salt.

4. A composition in accordance with claim 1 further characterized in that the acylated amine of (D) is prepared by the reaction of an olefin polymer-substituted succinic anhydride with more than an equivalent amount of an amine of the structure



in which  $n$  is an integer, A is selected from the group consisting of hydrogen, a hydrocarbon radical, and a hydroxyalkyl radical, and Q is a divalent aliphatic radical containing at least two carbon atoms.

5. A fluid composition adapted to form a protective coating on metals which contain as essential ingredients (A) from about 125 to about 200 parts of powdered zinc, (B) from about 10 to about 30 parts of an epoxy resin of 300-500 average molecular weight prepared by the reaction of a bis-(p-hydroxyphenyl) alkane with a chlorine-substituted terminal alkylene oxide, (C) from about 4 to about 16 parts of a zinc salt of the phosphorodithioic acid prepared by the reaction of a mixture of a monohydric alcohol and from 0.25 to 4.0 equivalents of a polyhydric alcohol with phosphorus pentasulfide, (D) from about 5 to about 15 parts of an oil-soluble acylated amine prepared by mixing and heating at a temperature of from about 80° C. to about 200° C., a polyisobutene-substituted succinic anhydride with from about 1.5 to about 4 equivalents of an ethylene amine, and (E) at least about 25 parts of a volatile solvent selected from the group consisting of petroleum hydrocarbon solvents, alcohols, ketones, lower chlorinated alkanes, aromatic hydrocarbons, and aliphatic ethers.

6. A fluid composition adapted to provide a protective coating for metals which contains as essential ingredients (A) from about 150 to about 175 parts of powdered zinc passing 325-mesh screen, (B) from about 14 to about 25 parts of an epoxy resin of 350-400 average molecular weight prepared by the reaction of 2,2-bis-(p-hydroxyphenyl)propane with epichlorohydrin, (C) from about 6 to about 10 parts of a zinc salt of the phosphorodithioic acid prepared by the reaction of a mixture of about equivalent amounts of isooctyl alcohol and dipropylene glycol with phosphorus pentasulfide (D) from about 8 to about 12 parts of an oil-soluble acylated amine prepared by mixing and heating at a temperature of from about 80° C. to about 200° C., a polyisobutene-substituted succinic anhydride wherein the polyisobutene has an average molecular weight of about 750 with about 4 equivalents of a mixture of diethylene triamine and triethylene, tetramine, and (E) from about 30 to about 70 parts of a volatile solvent consisting of a mixture of aromatic petroleum spirits and methyl isobutyl ketone.

#### References Cited by the Examiner

##### UNITED STATES PATENTS

|    |           |         |                |             |         |
|----|-----------|---------|----------------|-------------|---------|
| 45 | 2,820,723 | 1/1958  | Le Suer        | -----       | 117-132 |
|    | 2,858,323 | 10/1958 | Smith          | -----       | 260-561 |
|    | 2,861,907 | 11/1958 | Butler         | 260-461.113 | XR      |
|    | 2,970,972 | 2/1961  | Wear et al.    | 260-47      | XR      |
| 50 | 3,062,773 | 11/1962 | Rogier         | -----       | 260-18  |
|    | 3,075,932 | 1/1963  | Edwards et al. | -----       | 260-18  |

##### FOREIGN PATENTS

|         |        |                |
|---------|--------|----------------|
| 766,273 | 1/1957 | Great Britain. |
|---------|--------|----------------|

55 LEON J. BERCOVITZ, Primary Examiner.